

Aug. 30, 1932.

A. E. HARNSBERGER ET AL

1,874,743

METHOD OF PRODUCING CATALYTIC CORES

Original Filed Aug. 21, 1928

Fig. 1



Fig. 3



Fig. 4



Fig. 5



Inventor

A. E. Harnsberger  
C. L. Smith

By W. D. Maxwell

Attorney

## UNITED STATES PATENT OFFICE

AUDLEY E. HARNISBERGER AND CLYDE L. SMITH, OF CHICAGO, ILLINOIS, ASSIGNEES  
TO GYRO PROCESS COMPANY, OF DETROIT, MICHIGAN, A CORPORATION OF MICHIGAN

## METHOD OF PRODUCING CATALYTIC CORES

Original application filed August 21, 1928, Serial No. 301,152. Divided and this application filed December 14, 1929. Serial No. 414,167.

This invention relates to an improved type of catalytic core of the type used in connection with processes and apparatus for cracking petroleum oils. In certain of these processes oil is heated to substantially a state of vapor and is then passed through tubes or pipes for further heat treatment so that the temperature of the oils or vapors will be raised sufficiently to effect molecular decomposition thereof. It has been found in certain systems that by arranging within the tubes or pipes where the oil is heated to cracking temperatures, the conversion reactions are facilitated through bringing such vapors into contact with reaction promoting materials, among which may be mentioned ferrous oxide, although other materials are and have been used for this purpose.

It is desirable in such systems of oil cracking to maintain a uniform flow of oil vapor at constant velocity through the converting elements. For this reason it is undesirable to place the catalytic material in loose or bulk form in the converting elements for the reason that the flow of vapor is rendered ununiform and frequently the tubes or elements are clogged or blocked so that overheating is produced. In the cracking of petroleum oils time and temperature are the important factors, and the time factor must be as carefully controlled as the temperature factor. For this reason it has been proposed that cores composed of catalytic substances be provided, wherein the cores are composed of, for example, ferrous oxide mixed with a binder such as cement for the purpose of producing an elongated core possessing uniform diameter and of substantially solid formation. Such a core, in operation, possesses a considerably smaller diameter than the inside diameter of the tube or pipe, or other converting element in which it is situated, with the result that there remains an annular space in the converting element through which the vapors under heat treatment pass usually at high velocity.

The use of such cores, however, has demonstrated that under practical operating conditions they are very apt to burst, with the result that the tube or converting element is

obstructed and it is necessary to shut down temporarily the operation of the converter until the burst core or filler has been removed and a new one substituted. This is due to the fact that internal pressure is built up therein either by reason of high coefficient of expansion, the growth of the core or filler under high temperatures, or the building up of high gas pressure inside of the core.

We have found that by making the cores more porous and not a solid mass that the conditions mentioned above are largely overcome. One method of accomplishing this is to produce a mixture consisting of substantially ninety parts of iron oxide and cement and ten parts of sawdust, placing this mixture in a perforated pipe in a packed state and then subjecting the perforated pipe and its internal filler to a high temperature so as to drive off the moisture and to carbonize the sawdust. This results in a porous core which permits internal pressure to be readily removed or prevented with the result that the core is less apt to break or burst when subjected to the high temperatures found in the operation of oil conversion systems.

This application is a division of our previous application, Serial Number 301,152, filed August 21, 1928.

For a further understanding of the invention reference is to be had to the following description and the accompanying drawing wherein:

Figure 1 is a view in side elevation of a catalytic core formed in accordance with the present invention,

Figure 2 is a vertical sectional view taken through the core showing the latter positioned with a tube of the oil converter,

Figure 3 is a view in side elevation and partly in vertical section of a slightly modified form of core,

Figure 4 is a similar view of a further modified type of core,

Figure 5 is a view in side elevation of the perforated container in which the core is formed.

In accordance with the present invention, there is provided a core 1 consisting of an elongated body which is substantially round

55

65

70

75

80

85

90

95

100

in a cross section and made of any suitable weight, this being a factor which is regulated by the length of the converter element or pipe 2 in which the core is situated when 5 in operation in an oil conversion system. It will be observed that the core possesses an outside diameter which is substantially less than the inside diameter of the pipe 2, in order that there may be provided an annular 10 space 3 between the complementary walls of the core and pipe through which the oil vapors under treatment are passed. The cores may be supported in a central position co-extensive with the axis of the pipe 2 by means of 15 wire legs 4. The latter rest upon the bottom of the pipe 2 and serve to centralize and support the core axially within said pipe and at the same time offer the least resistance to the passage of the oil vapors through the 20 space 3.

The core is composed preferably of iron oxide, concrete or other cementitious materials which are mixed with sawdust or the like, that is to say, there is employed roughly 25 10 per cent of sawdust to 90 per cent of iron oxide and cement. These materials are placed while wet or moist in container 5 which consists preferably of a tubular or cylindrical metallic body suitably perforated 30 as at 6. The core materials are suitably packed in the container and then the latter is placed in a furnace and subjected to sufficiently high temperatures to drive off the moisture and to carbonize the sawdust content 35 thereof. This results in the production of an extremely porous core in which it will be practically impossible for gas to pocket or accumulate and which will therefore prevent the bursting of the cores and the premature destruction thereof when subjected to 40 the operating temperatures and conditions which prevail in the converting element or pipe 2 of the oil conversion system.

The second method for accomplishing similar results is to make the center of the core hollow, as shown in Figure 3. This can be accomplished by placing in the center of the container 5 a wooden rod or staff indicated at 7, around which is packed the concrete and ferrous oxide. This core is then subjected to 45 heat for the purpose of carbonizing the rod 7 to produce an axial passage within the core so that any internal pressure can be relieved through the center section or passage. The core shown in Figure 3 may also include in 50 the body thereof a certain percent of sawdust so that the walls of the core will be rendered porous.

This form of the invention is also exemplified in the construction disclosed in Figure 4 wherein during the manufacture of the core a small tube 8 of thin metal is inserted in the container and which in the operation of the core could easily collapse under abnormal 60 pressures or strains.

Through the provision of the above construction it will be seen that by rendering the material porous as disclosed provision is made to compensate for high internal pressures to prevent the fracture of such materials 70 and the perforate steel casing surrounding the same. As previously explained, these perforate steel casings were formerly filled solidly with the concrete and ferrous oxide with the result that when the cores or fillers 75 were placed in a converter tube and subjected to the high temperatures there prevailing, usually 1100° F., the tremendous stresses set up inside of these perforate pipes or cases 80 would result frequently in the bursting of the same. This difficulty is believed to be due principally to the growth of the material under the temperature causing high internal pressure. However, in accordance with the 85 present invention the filler or core is rendered porous by the use of the sawdust in the compositions thereof, and the resulting porosity produced by the construction results in relieving the strain since it gives room for expansion due to the growth of the material under 90 the influence of heat.

What is claimed is:

1. The method of producing catalytic cores for use in tubular oil heaters, which consists in producing a plastic mixture composed of a material possessing catalytic activity in oil cracking reactions, an organic substance and a cementitious material, molding said mixture while in said plastic state in the form of an elongated rod or core, and then subjecting said mixture to temperatures sufficiently high to effect the carbonization of said organic material and a hardening or setting of the mixture into a permanent rod-like form, whereby said rod or core possesses a 100 porous structure exposing large surface area of said catalytic material.

2. The method of producing catalytic cores for use in tubular oil heaters, which consists in producing a plastic mixture composed of a material possessing catalytic activity in oil cracking reactions, an organic substance and a cementitious material, molding said mixture in the form of an elongated rod or core, then subjecting said mixture to temperatures sufficiently high to effect the carbonization of said organic material and a hardening or setting of the mixture into a substantially porous permanent rod-like form, and releasing the volatiles from said mixture as rapidly as they are formed during the heating of said materials.

3. The method of producing catalytic cores for use in tubular reaction chambers which consists in producing a substantially plastic mixture composed of iron oxide, a carbonaceous and a cementitious material, molding said mixture while in said plastic state in the form of an elongated rod or core, and then subjecting said mixture to temperatures sufficiently 120 125 130

high to effect the burning of said carbonaceous material and the hardening or setting of the mixture into its desired permanent rod-like form, the burning of said carbonaceous material serving to render the finished rod or core substantially porous, whereby a large surface area of the ferrous oxide is exposed for reaction facilitating purposes.

In testimony whereof we affix our signatures.

10      AUDLEY E. HARNSBERGER.  
CLYDE L. SMITH.

15

20

25

30

35

40

45

50

55

60

65